

Sept. 16, 1958

L. G. S. BROOKER ET AL  
SENSITIZATION OF SILVER HALIDE EMULSIONS  
BY MEROCYANINES FROM TRIAZOLO BASES  
Filed June 25, 1956

2,852,384

**Fig. 1**



A= 3-ETHYL-[(2-ETHYL-1(2H)- $\Delta$ -TRIAZOLO[3,4-*b*] BENZO-  
THIAZOLYLIDENE) ETHYLIDENE] RHODANINE

**Fig. 2**



B= 3-ETHYL-5-[(2-METHYL-1(2H)- $\Delta$ -TRIAZOLO[3,4-*b*] BENZO-  
THIAZOLYLIDENE) ETHYLIDENE]-2-THIO-2,4-OXAZOLIDINEDIONE

**Fig. 3**



C= 5-[(7-CHLOR-2-ETHYL-1(2H)- $\Delta$ -TRIAZOLO[3,4-*b*] BENZOTHI-  
AZOLYLIDENE) ETHYLIDENE]-3-ETHYLRHODANINE

Leslie G.S. Brooker  
Earl J. Van Lare  
INVENTORS

BY  
Daniel J. Mayne,  
Lawrence H. Willis  
ATTORNEYS

# United States Patent Office

2,852,384

Patented Sept. 16, 1958

1  
2,852,384

## SENSITIZATION OF SILVER HALIDE EMULSIONS BY MEROCYANINES FROM TRIAZOLO BASES

Leslie G. S. Brooker and Earl J. Van Lare, Rochester, N. Y., assignors to Eastman Kodak Company, Rochester, N. Y., a corporation of New Jersey

Application June 25, 1956, Serial No. 593,615

12 Claims. (Cl. 96—102)

This invention relates to merocyanine dyes which are useful in optically sensitizing photographic silver halide emulsions, and a method for making such merocyanine dyes.

The merocyanine dyes of our invention can advantageously be represented by the following general formula:



wherein R represents an alkyl group, such as methyl, ethyl, n-propyl, isopropyl, n-butyl, isobutyl, allyl (vinylmethyl),  $\beta$ -ethoxyethyl, benzyl (phenylmethyl), etc. (e. g., an alkyl group of the formula  $C_mH_{2m+1}$  wherein  $m$  represents a positive integer of from 1 to 4), Z represents the non-metallic atoms necessary to complete a heterocyclic nucleus of the benzothiazole series or the quinoline series, n represents a positive integer of from 1 to 2, and Q represents the non-metallic atoms necessary to complete a heterocyclic nucleus containing from 5 to 6 atoms in the heterocyclic ring, such as those of the pyrazolone series (e. g., 3-methyl-1-phenyl-5-pyrazolone, 1-phenyl-5-pyrazolone, 1-(2-benzothiazolyl)-3-methyl-5-pyrazolone, etc.), those of the isoxazolone series (e. g., 3-phenyl-5(4H)-isoxazolone, 3-methyl-5(4H)-isoxazolone, etc.), those of the oxindole series (e. g., 1-alkyl-2,3-dihydro-2-oxindoles, etc.), those of the 2,4,6-triketohexahydropyrimidine series (e. g., barbituric acid or 2-thiobarbituric acid, as well as their 1-alkyl (e. g., 1-methyl, 1-ethyl, 1-n-propyl, 1-n-heptyl, etc.), or 1,3-dialkyl (e. g., 1,3-dimethyl, 1,3-diethyl, 1,3-di-n-propyl, 1,3-diisopropyl, 1,3-dicyclohexyl, 1,3-di( $\beta$ -methoxyethyl), etc.), or 1,3-diaryl (e. g., 1,3-diphenyl, 1,3-di( $p$ -chlorophenyl), 1,3-di( $p$ -ethoxycarbonylphenyl), etc.), or 1-aryl (e. g., 1-phenyl, 1-p-chlorophenyl, 1-p-ethoxycarbonylphenyl, etc.) or 1-alkyl-3-aryl (e. g., 1-ethyl-3-phenyl, 1-n-heptyl-3-phenyl, etc.) derivatives, those of the rhodanine series (i. e., 2-thio-2,4-thiazolidinedione series), such as rhodanine, 3-alkylrhodanines (e. g., 3-ethylrhodanine, 3-allylrhodanine, etc.) or 3-arylrhodanines (e. g., 3-phenylrhodanine, etc.), etc., those of the 2(3H)-imidazo[1,2- $\alpha$ ]pyridone series, those of the 5,7-dioxo-6,7-dihydro-5-thiazolo[3,2- $\alpha$ ]pyrimidine series (e. g., 5,7-dioxo-3-phenyl-6,7-dihydro-5-thiazolo[3,2- $\alpha$ ]pyrimidine, etc.), those of the 2-thio-2,4-oxazolidinedione series (i. e., those of the 2-thio-2,4(3H,5H)-oxazoledione series) (e. g., 3-ethyl-2-thio-2,4-oxazolidinedione, etc.), those of the thianaphthenone series (e. g., 3-(2H)-thianaphthenone, etc.), those of the 2-thio-2,5-thiazolidinedione series (i. e., the 2-thio-2,5(3H,4H)thiazoledione series) (e. g., 3-ethyl-2-thio-2,5-thiazolidinedione, etc.), those of the 2,4-thiazolidinedione series (e. g., 2,4-thiazolidinedione, 3-ethyl-2,4-thiazolidinedione, 3-phenyl-

2,4-thiazolidinedione, 3- $\alpha$ -naphthyl-2,4-thiazolidinedione, etc.), those of the thiazolidinone series (e. g., 4-thiazolidinone, 3-ethyl-4-thiazolidinone, 3-phenyl-4-thiazolidinone, 3- $\alpha$ -naphthyl-4-thiazolidinone, etc.), those of the 4-thiazolinone series (e. g., 2-ethylmercapto-4-thiazolinone, 2-alkylphenylamino-4-thiazolinones, 3-diphenylamino-4-thiazolinone, etc.), those of the 2-imino-2,4-oxazolinone (i. e., pseudohydantoin) series, those of the 2,4-imidazolidinedione (hydantoin) series (e. g., 2,4-imidazolidinedione, 3-ethyl-2,4-imidazolidinedione, 3-phenyl-2,4-imidazolidinedione, 3- $\alpha$ -naphthyl-2,4-imidazolidinedione, 1,3-diethyl-2,4-imidazolidinedione, 1-ethyl-3- $\alpha$ -naphthyl-2,4-imidazolidinedione, 1,3-diphenyl-2,4-imidazolidinedione, etc.), those of the 2-thio-2,4-imidazolidinedione (i. e., 2-thiohydantoin) series (e. g., 2-thio-2,4-imidazolidinedione, 3-ethyl-2-thio-2,4-imidazolidinedione, 3-phenyl-2-thio-2,4-imidazolidinedione, 3- $\alpha$ -naphthyl-2-thio-2,4-imidazolidinedione, 1,3-diethyl-2-thio-2,4-imidazolidinedione, 1-ethyl-3-phenyl-2-thio-2,4-imidazolidinedione, 1,3-diphenyl-2-thio-2,4-imidazolidinedione, etc.), those of the 5-imidazolinone series (e. g., 2-n-propylmercapto-5-imidazolinone, etc.), etc. (especially a heterocyclic nucleus containing 5 atoms in the heterocyclic ring, 3 of said atoms being carbon atoms, 1 of said atoms being a nitrogen atom, and 1 of said atoms being selected from the group consisting of a nitrogen atom, an oxygen atom, and a sulfur atom).

It is, therefore, an object of our invention to provide new merocyanine dyes. A further object is to provide methods for making these new dyes. Still another object is to provide new dye intermediates. A further object is to provide photographic silver halide emulsions sensitized with the new dyes of our invention. Other objects will become apparent from a consideration of the following description and examples.

According to our invention, we provide the dyes represented by Formula I above by condensing a compound selected from those represented by the following general formula:

II.



wherein R and Z each have the values given above and X represents an acid radical, such as chloride, bromide, iodide, perchlorate, benzenesulfonate, p-toluenesulfonate, methylsulfate, ethylsulfate, etc., together with a compound selected from those represented by the following general formula:

III.



wherein n and Q each have the values given above, R<sub>1</sub> represents a hydrogen atom or a carboxylic acyl group, such as acetyl, propionyl, butyryl, isobutyryl, benzoyl, toluoyl, etc. (e. g., a carboxylic acyl group containing from 2 to 7 carbon atoms), and R<sub>2</sub> represents an aryl group, such as phenyl, o-, m- and p-tolyl, etc. (e. g., a monocyclic aromatic group of the benzene series).

The condensations can advantageously be carried out in the presence of a basic condensing agent, such as the trialkylamines (e. g., triethylamine, tripropylamine, triisopropylamine, tributylamine, triisobutylamine, triamylamine, etc.), the N,N-dialkylanilines (e. g., N,N-dimethylaniline, N,N-diethylaniline, etc.), the N-alkylpiperidines (e. g., N-methylpiperidine, N-ethylpiperidine, etc.), etc.

An inert diluent, such as the lower aliphatic alcohols (e. g., ethanol, propanol, isopropanol, butanol, etc.), 1,4-dioxane, cyclohexane, pyridine, quinoline, etc., can also be employed. Heating accelerates the condensations, although temperatures varying from ambient temperature (ca. 25° C.) to the reflux temperature of the reaction mixture can be employed advantageously.

The intermediates represented by Formula II above can advantageously be prepared by heating together a base selected from those represented by the following general formula:

IV.



wherein Z has the values given above, with an alkyl salt represented by the following general formula:

V.



wherein R and X each have the values given above. Temperatures varying from about the temperature of the steam bath to about 200° C. can be employed.

The intermediates represented by Formula IV above can be prepared by condensing a compound selected from those represented by the following general formula:

VI.



wherein Z has the values given above, together with acetic anhydride in the presence of a strong acid, e. g., glacial acetic acid, phosphoric acid, etc. Where the condensation is slow, improved results can be obtained by first acetylating the hydrazino group of the compound of Formula VI, purifying the acetylated intermediate by crystallization, and completing the condensation by adding fresh acetic anhydride and strong acid, and heating under reflux. The carbocyclic ring of the compounds represented by Formula VI can contain simple substituents, such as chlorine, bromine, iodide, methoxyl, ethoxyl, methyl, ethyl, phenyl, etc. Intermediates represented by Formula VI above have been previously described in Brooker U. S. Patent 2,743,274, issued April 24, 1956, and Bayer et al. U. S. Patent 2,073,600, dated March 16, 1937.

Alternatively, the intermediates represented by Formula IV above can be prepared by condensing a compound selected from those represented by Formula VI above with an alkyl orthoacetate (e. g., methyl orthoacetate, ethyl orthoacetate, etc.). Heat accelerates these condensations and the addition of small amounts of an active solvent, such as pyridine, further accelerates the condensations. The foregoing method of preparing the intermediates represented by Formula IV above is particularly useful in those cases where it is desired to prepare intermediates having a substituent on the carbocyclic ring of the compounds represented by Formula IV.

The following examples will serve to illustrate more fully the manner whereby we practice our invention.

*Example 1.—3-ethyl-5-[(2-ethyl-1(2H)-s-triazolo[4,3-a]quinolylidene)ethylidene]rhodanine*



2 - ethyl - 1 - methyl - s - triazolo[4,3 - a]quinolinium iodide (1.7 g., 1 mol.), 5-acetanilidomethylene-3-ethylrhodanine (1.5 g., 1 mol.), pyridine (15 ml.) and triethylamine (0.5 g., 1 mol.) were refluxed together for one hour. After chilling, the dye was filtered off and washed with ethyl alcohol. After two recrystallizations from methyl alcohol, a 16% yield of reddish crystals with a blue reflex was obtained, M. P. 226-227° C. dec.

*Example 2.—3-ethyl-5-[(2-methyl-1(2H)-s-triazolo[3,4-b]benzothiazolylidene)ethylidene]rhodanine*



1-methyl-s-triazolo[3,4-b]benzothiazole (1.9 g., 1 mol.) and methyl p-toluenesulfonate (1.9 g., 1 mol.) were heated together at 160-170° C. for 3 hours. After cooling, 5-acetanilidomethylene-3-ethylrhodanine (3 g., 1 mol.), pyridine (10 ml.) and triethylamine (2 g., 2 mols.) were added, and the mixture was refluxed 30 minutes. After chilling, the dye was filtered off and washed with methyl alcohol. The crude dye was dissolved in pyridine and precipitated with methyl alcohol. A 23% yield of scarlet powder was obtained, M. P. 276-277° C. dec.

*Analysis.*—Calc'd for C<sub>16</sub>H<sub>14</sub>N<sub>4</sub>OS<sub>3</sub>: C, 51.3; H, 3.8. Found: C, 51.4; H, 3.7.

*Example 3.—3 - ethyl - 5 - [(2 - methyl - 1 (2H) - s - triazolo[3,4 - b]benzothiazolylidene)ethylidene] - 2-thio-2,4-oxazolidinedione*



1-methyl-s-triazolo[3,4-b]benzothiazole (1.9 g., 1 mol.) and methyl p-toluenesulfonate (1.9 g., 1 mol.) were heated together at 150-160° C. for three hours. After cooling, 5 - acetanilidomethylene - 3-ethyl-2-thio-2,4-oxazolidinedione (2.9 g., 1 mol.), pyridine (10 ml.) and triethylamine (2 g., 2 mols.) were added and the mixture was refluxed for twenty minutes. The reaction mixture was diluted to 200 ml. with methyl alcohol and then chilled. The crude dye was filtered off and washed with methyl alcohol. The dye was dissolved in pyridine and precipitated with methyl alcohol. A 54% yield of orange needles was obtained, M. P. 250-251° C. dec.

*Example 4.—3-ethyl-5-[(2-ethyl-1(2H)-s-triazolo[3,4-b]benzothiazolylidene)ethylidene]rhodanine*



1-methyl-s-triazolo[3,4-b]benzothiazole (1.9 g., 1 mol.) and diethyl sulfate (1.6 g., 1 mol.) were heated together at 150-160° C. for four hours. After cooling, 5-acetanilidomethylene-3-ethylrhodanine (3 g., 1 mol.), pyri-

dine (10 ml.) and triethylamine (2 g., 2 mols.) were added and the mixture refluxed for twenty minutes. The reaction mixture was diluted to 200 ml. with methyl alcohol and then chilled. The crude dye was filtered off and washed with methyl alcohol. The dye was dissolved in pyridine and precipitated with methyl alcohol. A 45% yield of fine, reddish-brown needles was obtained, M. P. 244-245° C. dec.

Example 5.—3-ethyl-5-[(2-ethyl-1-(2H)-s-triazolo[3,4-b]benzothiazolylidene)ethylidene]-1-phenyl-2-thiohydantoin



1-methyl-s-triazolo[3,4-b]benzothiazole (1.9 g., 1 mol.) and diethyl sulfate (1.6 g., 1 mol.) were heated together at 150-160° C. for four hours. After cooling, 5-acetanilidomethylene-3-ethyl-1-phenyl-2-thiohydantoin (3.6 g., 1 mol.), pyridine (10 ml.) and triethylamine (2 g., 2 mols.) were added and the mixture refluxed for thirty minutes. After cooling, the reaction mixture was treated with ether, the ether layer decanted off, and the residual oil washed again with ether. A small amount of ethyl alcohol was added and the oil became crystalline. The mixture was chilled and the solid filtered off and washed with ethyl alcohol. After two recrystallizations from methyl alcohol, the dye was obtained as brownish crystals in a 36% yield, M. P. 165-166° C. dec.

Example 6.—1,3-diethyl-5-[(2-ethyl-1-(2H)-s-triazolo[3,4-b]benzothiazolylidene)ethylidene]-2-thiobarbituric acid



1-methyl-s-triazolo[3,4-b]benzothiazole (1.9 g., 1 mol.) and diethyl sulfate (1.6 g., 1 mol.) were heated together at 150-160° C. for four hours. After cooling, 5-acetanilidomethylene-1,3-diethyl-2-thiobarbituric acid (3.45 g., 1 mol.), pyridine (10 ml.) and triethylamine (2 g., 2 mols.) were added and the mixture refluxed for thirty minutes. The reaction mixture was diluted to 200 ml. with methyl alcohol and then chilled. The crude dye was filtered off and washed with methyl alcohol. The dye was dissolved in pyridine and precipitated with methyl alcohol. A 40% yield of yellow needles was obtained M. P. 256-260° C. with previous shrinking.

Example 7.—4-[(2-ethyl-1-(2H)-s-triazolo[3,4-b]benzothiazolylidene)ethylidene]-3-methyl-1-p-sulfophenyl-5-pyrazolone



1-methyl-s-triazolo[3,4-b]benzothiazole (1.9 g., 1 mol.) and diethylsulfate (1.6 g., 1 mol.) were heated together

75

at 150-160° C. for four hours. After cooling, 4-anilino-methylene-3-methyl-1-p-sulfophenyl-5-pyrazolone (3.6 g., 1 mol.), pyridine (10 ml.) and triethylamine (2 g., 2 mols.) were added and the mixture refluxed for one and one-half hours. After cooling, the reaction mixture was treated with ether, the ether layer decanted off, and the residual oil washed again with ether. The oil remaining was dissolved in a small amount of ethyl alcohol and the solution made acid with conc. hydrochloric acid. After cooling, the crude dye was filtered off and washed with methyl alcohol. The dye was dissolved in methyl alcohol with the addition of triethylamine, the solution was filtered and the solution made acid with hydrochloric acid. The dye which separated was filtered off and washed with methyl alcohol. After repeating the above purification, the dye was obtained as brownish crystals in a 22% yield, M. P. 289-290° C. dec.

Example 8.—5-[(6-ethoxy-2-ethyl-1-(2H)-s-triazolo[3,4-b]benzothiazolylidene)ethylidene]-3-ethylrhodanine



35 6-ethoxy-1-methyl-s-triazolo[3,4-b]benzothiazole (1.17 g., 1 mol.) and diethyl sulfate (0.77 g., 1 mol.) were heated together at 150-160° C. for four hours. After cooling, 5-acetanilidomethylene-3-ethylrhodanine (1.53 g., 1 mol.), pyridine (10 ml.) and triethylamine (1 g., 2 mols.) were added and the mixture refluxed thirty minutes. The reaction mixture was diluted to 100 ml. with methyl alcohol and then chilled. The crude dye was filtered off and washed with methyl alcohol. The dye was dissolved in pyridine, the pyridine solution was filtered, and the dye precipitated with methyl alcohol. A 40 45 37% yield of fine orange needles was obtained, M. P. 240-241° C. dec.

Example 9.—5-[(7-chloro-2-ethyl-1-(2H)-s-triazolo[3,4-b]benzothiazolylidene)ethylidene]-3-ethylrhodanine



7-chloro-1-methyl-s-triazolo[3,4-b]benzothiazole (0.9 g., 1 mol.) and diethylsulfate (0.62 g., 1 mol.) were heated together at 150-160° C. for four hours. After cooling, 5-acetanilidomethylene-3-ethylrhodanine (1.3 g., 1 mol.), pyridine (5 ml.) and triethylamine (0.8 g., 2 mols.) were added and the mixture refluxed for thirty minutes. The reaction mixture was diluted to 100 ml. with methyl alcohol and then chilled. The crude dye was filtered off and washed with methyl alcohol. The dye was dissolved in pyridine, the pyridine solution was filtered, and the dye precipitated with methyl alcohol. An 18% yield of reddish brown needles was obtained, M. P. 242-243° C. dec.

Example 10.—3 - ethyl - 5 - [(2 - ethyl - 1(2H) - s - triazolo[3,4-b]benzothiazolylidene) - 2 - butenylidene] rhodanine



ethyl acetate. A 65% crude yield of colorless crystals was obtained, M. P. 155-158° C.

Example 13.—2-ethyl-1-methyl-s-triazolo[4,3-a]quinolinium iodide



1-methyl-s-triazolo[4,3-a]quinoline (9 g., 1 mol.) and ethyl iodide (12 g., 1½ mols.) were heated on a steam bath for 4 hours. The solid was ground in a mortar with acetone, filtered off and washed well with acetone. A 74% yield of tan crystals was obtained, M. P. 192-194° C. dec.

Example 14.—1-methyl-s-triazolo[3,4-b]benzothiazole



2-acetylhydrazinobenzothiazole (10.4 g., 1 mol.), acetic anhydride (50 ml.) and phosphoric acid (0.5 ml.) were refluxed together for 1 hour. The reaction mixture was poured into 400 ml. of water with stirring. The mixture was made alkaline with sodium carbonate solution, and the product filtered off and washed with water. After recrystallization from methyl alcohol an 81% yield of colorless crystals was obtained, M. P. 142-144° C.

Example 15.—2-acetylhydrazinobenzothiazole



2-hydrazinobenzothiazole (33 g., 1 mol.), acetic anhydride (40.8 g., 2 mols.) and acetic acid (100 ml.) were refluxed together for 1 hour. The acetic acid and acetic anhydride were removed on a steam bath under reduced pressure. The residue was dissolved in ethyl alcohol (200 ml.) and the solution made alkaline with 10% potassium carbonate solution. The mixture was cooled and the solid filtered off, washed with water and then with ethyl alcohol. After recrystallization from methyl alcohol, a 53% yield of colorless crystals was obtained, M. P. 213-215° C.

Analysis.—Calc'd for C<sub>9</sub>H<sub>9</sub>N<sub>3</sub>OS: C, 52.1; H, 4.3. Found: C, 52.3; H, 4.3.

As noted above we have found that our new dyes spectrally sensitize photographic silver halide emulsions when incorporated therein. The dyes are especially useful for extending the spectral sensitivity of the customarily employed gelatino-silver-chloride, gelatino-silver-chlorobromide, gelatino-silver bromide and gelatino-silver-bromide developing-out emulsions. To prepare emulsions sensitized with one or more of our new dyes, it is only necessary to disperse the dye or dyes in the emulsions. The methods of incorporating dyes in emulsions are simple and are known to those skilled in the art. In practice, it is convenient to add the dyes to the emulsions in the form of a solution in an appropriate solvent. Methanol or acetone has proved satisfactory as a solvent for most of our new dyes. Where the dyes are quite insoluble in methyl alcohol, a mixture of methyl alcohol and pyridine is advantageously

Example 12.—1-methyl-s-triazolo[4,3-a]quinoline.



2-quinolylhydrazine (31.8 g., 1 mol.), acetic anhydride (40.8 g., 2 mols.) and glacial acetic acid (100 ml.) were refluxed together for 1 hour. The reaction mixture was poured into 1 l. of water, neutralized with sodium carbonate, and then made strongly alkaline with sodium hydroxide. The mixture was extracted several times with ether to remove the unchanged quinolylhydrazine. On standing, a heavy oil, insoluble in water, ether, benzene and chloroform, slowly separated from the aqueous solution. After standing for two weeks, the oil became crystalline. It was filtered off and recrystallized from

employed as a solvent. The dyes are advantageously incorporated in the finished, washed emulsions and should be uniformly distributed throughout the emulsions. The particular solvent used will, of course, depend on the solubility properties of the particular dye.

The concentration of the dyes in the emulsions can vary widely, e. g., from 5 to 100 mg. per liter of flowable emulsion. The concentration of the dyes will vary according to the type of emulsion and according to the effect desired. The suitable and most economical concentration for any given emulsion will be apparent to those skilled in the art, upon making the ordinary tests and observations customarily used in the art of emulsion making. To prepare a gelatino-silver-halide emulsion sensitized with one or more of our new dyes, the following procedure is satisfactory.

A quantity of dye is dissolved in methyl alcohol or acetone (or a mixture of methyl alcohol and pyridine) and a volume of this solution, which may be diluted with water, containing from 5 to 100 mg. of dye, is slowly added to about 1000 cc. of gelatino-silver-halide emulsion, with stirring. Stirring is continued until the dye is thoroughly dispersed in the emulsion.

With most of our dyes, from 10 to 20 mg. of dye per liter of gelatino-silver-bromide or bromoiodide emulsion (containing about 40 g. of silver halide) suffices to produce the maximum sensitizing effect. With the finer grain emulsions, somewhat larger concentration of dye may be needed to produce the maximum sensitizing effect.

The above statements are only illustrative, as it will be apparent that the dyes can be incorporated in photographic emulsions by any of the other methods customarily employed in the art, e. g., by bathing a plate or film upon which an emulsion is coated in a solution of the dye in an appropriate solvent. However, bathing methods are ordinarily not to be preferred. Emulsions sensitized with the dyes can be coated on suitable supports, such as glass, cellulose derivative film, resin film or paper in the usual manner.

Photographic silver halide emulsions, such as those listed above, containing the sensitizing dyes of our invention can also contain such addenda as chemical sensitizers (e. g., sulfur sensitizers, such as allyl thiocarbamide, thiourea, allylisothiocyanate, cystine, etc.), various gold compounds (such as potassium chloroaurate, auric trichloride, etc.) (see U. S. Patents 2,540,085; 2,597,856; and 2,597,915, for example), various palladium compounds (such as palladium chloride (U. S. 2,540,086), potassium chloropalladate (U. S. 2,598,079), etc., or mixtures of such sensitizers), antifoggants (e. g., benzotriazole, nitrobenzimidazole, 5-nitroindazole, etc. (see Mees: "The Theory of the Photographic Process," Macmillan Pub., 1942, p. 460), or mixtures thereof), hardeners (e. g., formaldehyde (U. S. 1,763,533), chrome alum (U. S. 1,763,533), glyoxal (Germany 538,713), dibromacrolein (Great Britain 406,750), etc.), color couplers (e. g., such as those described in U. S. Patent 2,423,730, Spence and Carroll U. S. Patent 2,640,776, issued June 2, 1953, etc.), or mixtures of such addenda. Dispersing agents for color couplers, such as substantially water-insoluble, high boiling crystalloidal materials, such as those set forth in U. S. Patents 2,322,027 and 2,304,940, can also be employed in the above-described emulsions.

In the manner described above, a number of the dyes of our invention represented by Formula I above were separately incorporated in an ordinary gelatino-silver-chlorobromide emulsion, the dyes being added in the form of a solution in an organic solvent. The dyes were then thoroughly incorporated in the emulsions by stirring. After a short digestion, the emulsions were coated onto ordinary cellulose acetate film supports and the coatings exposed in a spectrograph and sensitometer and then developed in the usual way. The sensitizing range

and maximum absorption for several of the dyes are indicated in the following table.

| 5  | Dye of Example | Range in mμ. | Max. in mμ. |
|----|----------------|--------------|-------------|
| 3  |                | to 560       | 530         |
| 4  |                | to 620       | 560         |
| 5  |                | 470-570      | 535         |
| 6  |                | to 510       | 480         |
| 8  |                | to 615       | 565         |
| 9  |                | to 615       | 565         |
| 10 |                | to 680       | 510, 610    |

The accompanying drawing further illustrates our invention. Each figure is a diagrammatic reproduction of a wedge spectrogram showing the sensitivity of an ordinary gelatino-silver-bromide emulsion containing one of the sensitizing dyes represented by Formula I above. In Fig. 1, the curve depicts the sensitivity of an ordinary gelatino-silver-bromide emulsion sensitized with 3-ethyl-5-[(2-ethyl-1(2H)-s-triazolo[3,4-b]benzothiazolylidene)ethylidene]rhodanine. In Fig. 2, the curve depicts the sensitivity of an ordinary gelatino-silver-bromide emulsion sensitized with 3-ethyl-5-[(2-methyl-1(2H)-s-triazole[3,4-b]benzothiazolylidene)ethylidene]-2-thio-2,4-oxazolidinedione. In Fig. 3, the curve depicts the sensitivity of an ordinary gelatino-silver-bromide emulsion sensitized with 5-[(7-chloro-2-ethyl-1(2H)-s-triazolo[3,4-b]benzothiazolylidene)ethylidene]-3-ethylrhodanine.

This application is a continuation-in-part of our pending application Serial No. 451,062, filed August 19, 1954, now United States Patent 2,786,054, issued March 19, 1957.

What we claim as our invention and desire secured by Letters Patent of the United States is:

1. A photographic silver halide emulsion sensitized with a merocyanine dye selected from those represented by the following general formula:



wherein R represents a lower alkyl group, n represents a positive integer of from 1 to 2, and Q represents the non-metallic atoms necessary to complete a heterocyclic nucleus of the rhodanine series.

2. A photographic silver halide emulsion sensitized with a merocyanine dye selected from those represented by the following general formula:



wherein R represents a lower alkyl group, n represents a positive integer of from 1 to 2, Z represents the non-metallic atoms necessary to complete a heterocyclic nucleus of the benzothiazole series and Q represents the non-metallic atoms necessary to complete a heterocyclic nucleus of the rhodanine series.

3. A photographic silver halide emulsion sensitized with

11

a merocyanine dye selected from those represented by the following general formula:



wherein R represents a lower alkyl group, n represents a positive integer of from 1 to 2, Z represents the non-metallic atoms necessary to complete a heterocyclic nucleus of the benzothiazole series and Q represents the non-metallic atoms necessary to complete a heterocyclic nucleus of the 2-thio-2,4-oxazolidinedione series.

4. A photographic silver halide emulsion sensitized with a merocyanine dye selected from those represented by the following general formula:



wherein R represents a lower alkyl group, n represents a positive integer of from 1 to 2, Z represents the non-metallic atoms necessary to complete a heterocyclic nucleus of the benzothiazole series and Q represents the non-metallic atoms necessary to complete a heterocyclic nucleus of the 2-thio-2,4-imidazolidinedione series.

5. A photographic silver halide emulsion sensitized with a merocyanine dye selected from those represented by the following general formula:



wherein R represents a lower alkyl group, n represents a positive integer of from 1 to 2, Z represents the non-metallic atoms necessary to complete a heterocyclic nucleus of the benzothiazole series and Q represents the non-metallic atoms necessary to complete a heterocyclic nucleus of the 2,4,6-triketohexahydropyrimidine series.

6. A photographic silver halide emulsion sensitized with a merocyanine dye selected from those represented by the following general formula:



wherein R represents an alkyl group, n represents a positive integer of from 1 to 2, Z represents the non-metallic atoms necessary to complete a heterocyclic nucleus selected from the group consisting of those of the benzothiazole series and those of the quinoline series, and Q represents the non-metallic atoms necessary to complete a heterocyclic nucleus containing from 5 to 6 atoms in the heterocyclic ring.

7. A photographic gelatino-silver-halide emulsion sensitized with a merocyanine dye selected from those represented by the following general formula:



wherein R represents a lower alkyl group, n represents a positive integer of from 1 to 2, Z represents the non-metallic atoms necessary to complete a heterocyclic nucleus selected from the group consisting of those of the benzothiazole series and those of the quinoline series, and Q represents the non-metallic atoms necessary to complete a heterocyclic nucleus selected from the group consisting of those of the pyrazolone series, those of the isoxazolone series, those of the oxindole series, those of the 2,4,6-triketohexahydropyrimidine series, those of the rhodanine series, those of the 2(3H)-imidazo[1,2- $\alpha$ ]-pyridone series, those of the 5,7-dioxo-6,7-dihydro-5-thiazo[3,2- $\alpha$ ]pyrimidine series, those of the 2-thio-2,4-oxazolidinedione series, those of the thianaphthenone series, those of the 2-thio-2,5-thiazolidinedione series, those of the 2,4-thiazolidinedione series, those of the thiazolidinone series, those of the 4-thiazolinone series, those of the 2-imino-2,4-oxazolinone series, those of the 2-thio-2,4-imidazolidinedione series, those of the 2,4-imidazolidinedione series, and those of the 5-imidazolinone series.

8. A photographic silver halide emulsion sensitized with the merocyanine dye represented by the following formula:



9. A photographic silver halide emulsion sensitized with the merocyanine dye represented by the following formula:



10. A photographic silver halide emulsion sensitized with the merocyanine dye represented by the following formula:



11. A photographic silver halide emulsion sensitized with the merocyanine dye represented by the following formula:



12. A photographic silver halide emulsion sensitized

13

with the merocyanine dye represented by the following formula:



5

14

|           |                |               |
|-----------|----------------|---------------|
| 2,177,401 | Brooker        | Oct. 24, 1939 |
| 2,572,961 | Thompson       | Oct. 30, 1951 |
| 2,705,713 | Kendall et al. | Apr. 5, 1955  |
| 2,706,193 | Sprague        | Apr. 12, 1955 |

## OTHER REFERENCES

- Chemical Abstracts, 16, 3101 (abstract of Brit. Med. Journal, 1922, I, 514-5).  
 Chemical Abstracts, 19, 530 (abstract of Proc. Roy. Soc., London, 96B, 317-33, 1924).

## References Cited in the file of this patent

## UNITED STATES PATENTS

2,078,233 Brooker ----- Apr. 27, 1937 15